

## UNITED STATES PATENT OFFICE

2,460,252

## LEAD-TIN ALLOY PLATING

Arthur H. Du Rose, Euclid, and John D. Little, Lakewood, Ohio, assignors to The Harshaw Chemical Company, Elyria, Ohio, a corporation of Ohio

No Drawing. Application February 9, 1946,  
Serial No. 646,712

5 Claims. (Cl. 204—43)

1

This invention relates to lead-tin alloy plating and more specifically to a method of and means for causing preferential deposition of tin whereby the solution may have a smaller concentration with respect to tin than normally would be required for producing a co-deposit containing a given percentage of tin.

We are aware that prior to our invention co-deposits of lead and tin have been made. Accordingly we do not claim lead-tin alloy plating broadly. It is obvious, however, that if a plating solution containing only a small concentration of tin can be caused to deposit relatively more tin than lead as compared to previous solutions and at the same time produce adherent, impervious deposits suitable for protective coatings, a definite advantage will be gained in that the drag-out loss of the relatively expensive tin will be reduced.

We have now discovered a class of addition agents which may be added to fluoborate or sulfamate solutions of lead-tin electrolytes containing 5 parts of tin or less per 100 parts of lead by weight and which will cause preferential deposition of tin from such solutions. The class of addition agents referred to consists of the mono-, di-, and tri-hydroxy benzenes, the mono-, di- and tri-hydroxy diphenyls and the chloro, bromo, amino, methyl, ethyl, propyl and isopropyl substitution products of the above named addition agents wherein the named substituents are connected to ring carbon. Specific examples of the class which have been found to produce preferential deposition of tin are resorcinol, catechol, hydroquinone, pyrogallol, phloroglucinol, phenol, cresol, p-amino phenol, 2,4,5,6 trichlorophenol, o-amyl phenol, o-bromo phenol, 2,4-dihydroxy-diphenyl.

We have found that addition agents of the above group are effective in commercial plating solutions of the fluoborate and sulfamate types. The corresponding hydroxy naphthalenes are effective in the higher concentrations of tin but where the tin calculated as Sn is less than 5 parts

by weight to 100 parts by weight of lead calculated as Pb, the deposit is defective as a protective coating as hereinafter indicated. Preferred solution compositions for these types of solutions are as follows:

## Fluoborate solution

|                                                                                                                                                                                                                                                                    | Grams/Liter         |
|--------------------------------------------------------------------------------------------------------------------------------------------------------------------------------------------------------------------------------------------------------------------|---------------------|
| Lead (in the form of the fluoborate),                                                                                                                                                                                                                              | 10 99% to 95%       |
| Tin (in the form of the fluoborate),                                                                                                                                                                                                                               | 100 to 400 1% to 5% |
| Fluoboric acid                                                                                                                                                                                                                                                     | 10 to 200           |
| Glue                                                                                                                                                                                                                                                               | 0.2 to 1.5          |
| 15 An addition agent of the class consisting of mono-, di-, and tri-hydroxy benzenes and diphenyls and their chloro, bromo, amino, methyl, ethyl, propyl and isopropyl derivatives wherein the substituents are on ring carbon and mixtures of a plurality thereof | 0.2 to 5            |
| 20 Water                                                                                                                                                                                                                                                           | Remainder           |

## Sulfamate solution

|                                      | Grams/Liter         |
|--------------------------------------|---------------------|
| Lead (in the form of the sulfamate), | 10 99% to 95%       |
| Tin (in the form of the sulfamate),  | 100 to 250 1% to 5% |
| Sulfamic acid to give pH             | 1 to 1.5            |
| Glue                                 | 0 to 1.5            |

|                                                                                                                                                                                                                                                                    |            |
|--------------------------------------------------------------------------------------------------------------------------------------------------------------------------------------------------------------------------------------------------------------------|------------|
| 35 An addition agent of the class consisting of mono-, di-, and tri-hydroxy benzenes and di-phenyls and their chloro bromo, amino, methyl, ethyl, propyl and isopropyl derivatives wherein the substituents are on ring carbon and mixtures of a plurality thereof | 0.2 to 1.5 |
| 40 Water                                                                                                                                                                                                                                                           | Remainder  |

The following table showing specific examples

from actual practice will serve to illustrate the invention:

*Grams per liter of solution except as noted  
(remainder water)*

| Example No.                                         | 1     | 2     | 3     | 4     | 5     | 6     | 7     | 8     | 9     | 10    | 11    | 12    | 13    | 14    | 15    | 16     |
|-----------------------------------------------------|-------|-------|-------|-------|-------|-------|-------|-------|-------|-------|-------|-------|-------|-------|-------|--------|
| Lead Fluoborate (Pb Content)                        | 263   | 265   | 265   | 265   | 265   | 265   | 265   | 265   | 265   | 265   | 265   | 265   | 265   | 265   | 265   | -----  |
| Tin Fluoborate (Sn Content)                         | 7.5   | 7.5   | 7.5   | 7.5   | 7.5   | 7.5   | 7.5   | 7.5   | 7.5   | 7.5   | 7.5   | 7.5   | 7.5   | 7.5   | 7.5   | -----  |
| Fluoboric Acid                                      | 102.2 | 102.2 | 102.2 | 102.2 | 102.2 | 102.2 | 102.2 | 102.2 | 102.2 | 102.2 | 102.2 | 102.2 | 102.2 | 102.2 | 102.2 | 168.8  |
| Lead Sulfamate (Pb Content)                         | ----- | ----- | ----- | ----- | ----- | ----- | ----- | ----- | ----- | ----- | ----- | ----- | ----- | ----- | ----- | 7.5    |
| Tin Sulfamate (Sn Content)                          | ----- | ----- | ----- | ----- | ----- | ----- | ----- | ----- | ----- | ----- | ----- | ----- | ----- | ----- | ----- | 1.3 pH |
| Sulfamic Acid (To give pH of)                       | ----- | ----- | ----- | ----- | ----- | ----- | ----- | ----- | ----- | ----- | ----- | ----- | ----- | ----- | ----- | 0.4    |
| Glue                                                | 0.8   | 0.8   | 0.8   | 0.8   | 0.8   | 0.8   | 0.8   | 0.8   | 0.8   | 0.8   | 0.8   | 0.8   | 0.8   | 0.8   | 0.8   | 1.3 pH |
| Resorcinol                                          | 0.5   | 2.0   | ----- | ----- | ----- | ----- | ----- | ----- | ----- | ----- | ----- | ----- | ----- | ----- | ----- | -----  |
| Catechol                                            | ----- | 0.5   | 3.0   | ----- | ----- | 0.5   | 3.0   | ----- | ----- | ----- | ----- | ----- | ----- | ----- | ----- | -----  |
| Hydroquinone                                        | ----- | ----- | ----- | ----- | ----- | 0.5   | 3.0   | ----- | 0.5   | 3.0   | ----- | ----- | ----- | ----- | ----- | -----  |
| Pyrogallol                                          | ----- | ----- | ----- | ----- | ----- | ----- | ----- | ----- | ----- | ----- | ----- | ----- | ----- | ----- | ----- | -----  |
| Phloroglucinol                                      | ----- | ----- | ----- | ----- | ----- | ----- | ----- | ----- | ----- | ----- | ----- | ----- | ----- | ----- | ----- | -----  |
| Phenol                                              | ----- | ----- | ----- | ----- | ----- | ----- | ----- | ----- | ----- | ----- | 0.5   | 3.0   | ----- | 1.0   | ----- | -----  |
| Naphthol                                            | ----- | ----- | ----- | ----- | ----- | ----- | ----- | ----- | ----- | ----- | ----- | ----- | ----- | 0.4   | ----- | -----  |
| Cresol                                              | ----- | ----- | ----- | ----- | ----- | ----- | ----- | ----- | ----- | ----- | ----- | ----- | ----- | 0.4   | ----- | 0.4    |
| 3,4 dihydroxydiphenyl                               | ----- | ----- | ----- | ----- | ----- | ----- | ----- | ----- | ----- | ----- | ----- | ----- | ----- | ----- | ----- | 0.4    |
| Orthobromophenol                                    | ----- | ----- | ----- | ----- | ----- | ----- | ----- | ----- | ----- | ----- | ----- | ----- | ----- | ----- | ----- | 0.4    |
| <i>Percentage by weight</i>                         |       |       |       |       |       |       |       |       |       |       |       |       |       |       |       |        |
| Tin in deposit                                      | 2.45  | 4.47  | 1.81  | 3.46  | 2.26  | 4.22  | 1.65  | 3.90  | 6.44  | 7.08  | 2.5   | 4.75  | 14.86 | 4.31  | 2.86  | 1.37   |
| Tin in deposit in absence of special addition agent | 0.25  | 0.25  | 0.25  | 0.25  | 0.25  | 0.25  | 0.25  | 0.25  | 0.25  | 0.25  | 0.25  | 0.25  | 0.25  | 0.25  | 0.21  | 0.15   |

<sup>1</sup> Powdery deposit. Not suitable for use as a protective coating.

This application is a continuation-in-part of our co-pending application Serial No. 569,262, filed December 21, 1944, which has become abandoned.

Having thus described our invention, what we claim is:

1. An aqueous, acid lead-tin plating solution essentially consisting of from 100 to 400 grams per liter combined concentration of lead and tin ions, negative ions of the class consisting of fluoborate and sulfamate and an addition agent effective to cause increased deposition of tin in proportion to lead deposited, the concentration of tin ions being from 1% to 5% of the combined weight of lead and tin ions, and said addition agent being present to the extent of from 0.2 to 5 grams per liter and being selected from the class consisting of resorcinol, catechol, hydroquinone, pyrogallol, phloroglucinol, phenol, naphthol, cresol, 3,4 dihydroxydiphenyl, orthobromophenol, p-amino phenol and o-ethyl phenol.

2. The invention according to claim 1 wherein said addition agent is resorcinol.

3. The invention according to claim 1 wherein said addition agent is phenol.

4. The invention according to claim 1 wherein said addition agent is hydroquinone.

5. The invention according to claim 1 wherein said solution also contains from 0.2 to 1.5 grams per liter of glue.

ARTHUR H. DU ROSE.  
JOHN D. LITTLE.

#### REFERENCES CITED

35 The following references are of record in the file of this patent:

#### UNITED STATES PATENTS

40 Number Name Date  
Re. 12,301 Betts ----- Jan. 3, 1905  
2,318,592 Cupery ----- May 11, 1943

#### FOREIGN PATENTS

45 Number Country Date  
329,346 Great Britain ----- May 16, 1930

#### OTHER REFERENCES

50 Transactions of Electrochemical Society, vol. 76, pp. 371-382 (1939).

Transactions of Electrochemical Society, vol.

40, pp. 296-299 (1921).

Chemical Abstracts, vol. 38, p. 2571 (1944).